

## UNITED STATES PATENT OFFICE

2,214,444

## PROCESS FOR TREATING MINERAL OILS

Kegham A. Varteressian, State College, Pa.

No Drawing. Application March 2, 1937,  
Serial No. 128,618

8 Claims. (Cl. 252—53)

This invention pertains generally to the improvement of oils and pertains particularly to the stabilization thereof.

This invention pertains more particularly to the stabilization of lubricating oils intended for motor car use.

The result of improvements in the automobile motor to develop more power at higher operating temperatures with units occupying 10 smaller space, has been to place a much greater demand upon motor oils.

While commercial motor oils as a rule and particularly those made from Pennsylvania grade crudes are composed of highly inert substances 15 capable of heavy duty performance without substantial change in chemical composition, yet extreme service conditions, particularly when accompanied by high temperatures, are sometimes capable of causing undesirable chemical and/or 20 physical changes as evidenced, for instance, by the corrosion of certain types of bearings.

This invention is based upon the discovery that the stability of oils in general, and particularly those derived from Pennsylvania grade 25 crudes is materially improved upon the addition to said oil of a relatively small amount of a new stabilizing substance made by treating a phenol and particularly a simple phenol such as carbolic acid with arsenious chloride, preferably in 30 stoichiometric proportions such as would be required for instance in making triphenyl arsenite.

The following will illustrate the manufacture of this new stabilizing substance.

To 3 mols of phenol (carbolic acid) is added 1 35 mole of arsenious chloride, preferably with a slight addition of heat, say for instance sufficient to cause the reaction to take place at 50° C.

The reaction which takes place is accompanied by the evolution of a gaseous substance which is 40 thought to be at least chiefly hydrogen chloride.

After the reaction is complete the dissolved 45 gas is preferably removed by any suitable means known in the art.

In case phenol is used as a starting material 45 the resulting molecule is thought to contain three benzene rings, each linked to a single arsenic atom by means of an oxygen atom and will be hereinafter referred to as triphenyl arsenite.

In case cresol is used as a starting material 50 each of the three benzene rings is thought to contain a methyl group and the resulting substance will be hereinafter referred to as tricresyl arsenite.

When my new stabilizing substance is added 55 to a lubricating oil for instance to the extent of

0.5 percent by weight it prevents the corrosion of certain types of bearings as shown by the following test.

150 cubic centimeters of oil to be tested is placed in a glass test tube and raised to 341° F. Bearing sections are placed in the oil on glass hooks and a strip of copper having an area of 21 square centimeters is added to catalyze oxidation of the oil and thereby increase the severity of the test. 5 liters of air are passed through the 10 oil per hour. At definite time intervals the bearings are removed, cleaned and weighed. The loss in weight after cleaning is taken as a measure of the degree of corrosion.

To illustrate the stabilizing qualities of my new 15 stabilizing substance an untreated neutral oil was subjected to the foregoing test in the presence of a cadmium-nickel alloy bearing section having an area of 21 square centimeters. At the end of 12 hours the bearing section showed a loss due to 20 corrosion of approximately 100 milligrams.

This same oil was treated with 0.5 percent by weight of triphenyl arsenite followed by thorough mixing and when subjected to the same test for a period of 12 hours there was no loss in weight of 25 the cadmium-nickel bearing section due to corrosion.

The stabilizing effect of my new stabilizing substance is thus made clearly evident.

In view of the fact that the above test is extremely severe it follows that good results may be produced upon the addition of smaller quantities of the stabilizing substance. On the other hand, if desired, larger quantities may be added.

No difficulties have been experienced in bringing 35 larger quantities of the stabilizing substance into solution in the oil. However, if desired, solubilizing agents may be added.

It is to be understood that the foregoing description of a manner of making the stabilizing 40 substance is by way of illustration and not of limitation.

A variety of substances may be used as starting materials in the manufacture of the stabilizing substance, or other means may be employed 45 for building up the stabilizing molecule.

Further evidence of the stabilizing effects of my new stabilizing substance appears to reside in the improvement in other lubricating qualities.

Oils treated in accordance with this invention 50 may be used for any other purpose such as insulating oils for transformers, cables, etc., or for other lubricating purposes.

In the claims the term "lubricating oil" when referred to is intended to mean a petroleum oil 55

of a viscous character, that is, an oil having a viscosity of the order of 50 Saybolt seconds at 100° F. or more and regardless of the use to which such oil is put.

5 While procedure for the purpose of carrying out the invention has been particularly described it is to be understood that this is by way of illustration. Therefore changes, omissions, additions, substitutions, and/or modifications may be made 10 within the scope of the claims without departing from the spirit of the invention which is intended to be limited only as required by the prior art.

I claim:

1. A process for stabilizing a lubricating oil 15 comprising adding to said oil a quantity sufficient to inhibit corrosion of a stabilizing substance resulting from attaching three phenolate groups to a single arsenic atom.

2. A process for stabilizing a lubricating oil 20 comprising adding to said oil in quantity sufficient to inhibit corrosion triphenyl arsenite.

3. A process for stabilizing a lubricating oil comprising adding to said oil in quantity sufficient to inhibit corrosion tricresyl arsenite.

25 4. A process for stabilizing a hydrocarbon lubricating oil of a character normally tending to

corrode alloys having the corrosion susceptibility of cadmium-nickel alloys when continuously applied to the surface thereof under service conditions, comprising incorporating with said oil triphenyl arsenite in at least corrosion inhibiting 5 proportions.

5. A lubricating oil having in solution therein a quantity sufficient to inhibit corrosion of a substance resulting from attaching three phenolate groups to a single arsenic atom. 10

6. A lubricating oil having in solution therein triphenyl arsenite in quantity sufficient to inhibit corrosion.

7. A lubricating oil having in solution therein tricresyl arsenite in quantity sufficient to inhibit 15 corrosion.

8. Mineral oil composition comprising a hydrocarbon lubricating oil of a character normally tending to corrode alloys having the corrosion susceptibility of cadmium-nickel alloys 20 when continuously applied to the surface thereof under service conditions, and triphenyl arsenite incorporated with said oil in at least corrosion inhibiting proportions.

25 KEGHAM A. VARTERESSIAN.